

1

3,189,457

**SENSITIZED PHOTOGRAPHIC EMULSIONS CONTAINING QUATERNARY AMMONIUM COMPOUNDS**

Donald M. Burness, Rochester, N.Y., assignor to Eastman Kodak Company, Rochester, N.Y., a corporation of New Jersey

No Drawing. Filed Sept. 11, 1961, Ser. No. 137,035  
9 Claims. (Cl. 96—107)

This invention relates to photographic emulsions, and, more particularly, photographic emulsions of the silver halide type. It is known that the inherent sensitivity of photographic silver halide emulsions (whether spectrally sensitized or not) can be increased, and there has been constant effort to produce higher and higher speeds in photographic emulsions. For example, it is known that the speed of gelatino silver halide emulsions can be enhanced by an extended digestion or ripening of the emulsion. It is also known that the speed of silver halide emulsions (spectrally sensitized or not) can be enhanced by incorporating into the emulsions compounds containing an atom of the sulfur group directly joined by a double bond to a single metalloid atom to which is attached another group of atoms; for example, allyl isothiocyanate and allyl thiourea.

More recently, it has been found that the speed of photographic silver halide emulsions (whether spectrally sensitized or not) can be increased by incorporating in the emulsions a cationic surface active substance of the quaternary ammonium type. The speed increases thus obtainable are ordinarily complementary to the speeds obtainable by the prior methods. Many of the more active sensitizers, particularly of the quaternary ammonium type, have been double enders; that is they must contain two of the requisite quaternary ammonium functions in order to obtain reasonably high activity.

A difficulty encountered with several sensitizers is that the substances used to sensitize the emulsion appear to diffuse to a greater or less extent from the emulsions with the result that their effect upon the photographic emulsion may be decreased.

One object of my invention is to provide photographic emulsions chemically sensitized with quaternary ammonium compounds; another object is to provide quaternary ammonium compounds which diffuse, if any, only to a small extent into the film base upon which the emulsion is coated. Other objects of my invention will appear herein.

We have found that compounds useful for chemically sensitizing silver halide emulsions can be represented by the general formula:



where Y is an alkyl mercapto group of 6-30 carbon atoms or a secondary or a tertiary amino group containing a linear chain of 10-30 carbon atoms, R represents lower alkyl groups of 1-4 carbon atoms, and X is a suitable anion, or where as bis compound such as a dimercaptan or diamine is used in their preparation by a compound having the formula:



wherein Z is alkylene dimercapto or alkylene diamino, the chain connecting the end S or N being either straight ali-

2

phatic carbon chain or an aliphatic hetero chain, but in either case of at least 4 carbon atoms. These compounds are employed as sensitizers in photographic emulsions in concentrations therein not more than 4 g. per g. mole of silver halide in the photographic emulsion. In most instances, a satisfactory concentration of sensitizer is found between .2 g. and 3 g. per g. mole of silver halide. Compositions in accordance with the invention are prepared by adding to an ordinary aqueous silver halide emulsion, with or without other sensitization, the desired amount of the sensitizing material, such as in solution or suspension in water.

The preparation of sensitizers in accordance with my invention is conveniently carried out in excellent yield by reacting a quaternary ammonium epoxide with an appropriate amine or mercaptan. Some amines which are useful in preparing compounds in accordance with my invention are those having formulas such as



20 Alkyl substituted amines such as  $\text{C}_{14}\text{H}_{29}\text{NHCH}_3$  may also be employed. Some mercaptans which are useful for reacting with a quaternary ammonium epoxide to give sensitizers useful in my invention are  $\text{C}_8\text{H}_{17}\text{SH}$ ,  $\text{C}_{14}\text{H}_{33}\text{SH}$ ,  $\text{C}_6\text{H}_{13}\text{SH}$  and  $\text{C}_{12}\text{H}_{25}\text{SH}$ . If desired, amines or mercaptans having greater numbers of carbon atoms also show useful properties for sensitizing silver halide photographic emulsions.

25 In the preparation of bis compounds useful as sensitizers dimercapto compounds suitable for reacting with quaternary ammonium epoxides to prepare sensitizers are for example:



35 and the like.

30 Examples of diamino compounds suitable for reacting with quaternary ammonium epoxides to prepare sensitizers are:



40 and the like.

45 Some of the quaternary ammonium epoxides which may be reacted to form sensitizers in accordance with my invention are: 2,3-epoxypropyltrimethylammonium p-toluenesulfonate, 2,3-epoxypropyltrimethylpropylammonium p-toluenesulfonate, 2,3-epoxypropyltrimethylpropylammonium p-toluenesulfonate.

50 The preparation of sensitizing compounds of the mono-quaternary ammonium type for use in compositions in accordance with my invention is conveniently carried out in excellent yield by the reaction of a quaternary ammonium epoxide with an amine or mercaptan in accordance with the following equations:



65 R being alkyl groups of 1-4 carbon atoms, R' being alkyls as of  $\text{C}_6\text{-C}_{30}$  (mercaptan) or  $\text{C}_{10}\text{-C}_{30}$  (amine), R'' being either hydrogen or alkyl of 1-4 carbon atoms and X

being any suitable anion such as p-toluenesulfonate, perchlorate or the like.

For the preparation of sensitizing compounds of the bisquaternary ammonium type the dimercaptan or diamine is reacted with the quaternary ammonium epoxide to result in a compound having the formula



where R is alkyl of 1-4 carbon atoms, X<sup>-</sup> is a suitable anion and Z is an aliphatic chain containing at least 4 carbon atoms with or without hetero atoms such as sulfur, nitrogen or oxygen in the chain.

The following example illustrates the preparation of a sensitizing compound in accordance with my invention:

#### EXAMPLE 1

80 g. of 3-dimethylamino 1,2-epoxypropane prepared by the method described by Gilman and Fullhart, JACS 71, 1430 (1949), in solution in 600 ml. of dry benzene was mixed with 150 g. of methyl p-toluenesulfonate over a 10-minute period at 30-35° C. The mixture was allowed to stand at 25° C. overnight whereupon it was filtered and recrystallized from acetone to give 189 g. of colorless plate-formed crystals. 11.5 g. of the epoxypropyltrimethylammonium p-toluenesulfonate thus prepared was dissolved in 25 ml. of methanol which was added to a solution consisting of 14.8 g. of dodecylamine in 25 ml. of methanol. While the addition was taking place over a half-hour period, the mass was stirred and heated to 45° C. It was then maintained at this temperature with stirring for 18 hours. The solvent was removed, the product was stirred with ether and filtered. Recrystallization from acetonitrile gave 13.8 g. of colorless crystals of 3-n-dodecylamino-2-hydroxypropyl trimethylammonium p-toluenesulfonate.

Similar preparations were carried out of a number of similar compounds in like fashion, which compounds were separated out and analyzed. The compounds prepared, their yield, the melting points and formulas of the finished product are listed in the following table:

#### Quaternary salts,



from reaction of 2,3-epoxypropyltrimethylammonium p-tosylate with amines and mercaptans

| Reactant, YH                                                   | Yield, Percent | M.P., °C. | Formula                                                         |
|----------------------------------------------------------------|----------------|-----------|-----------------------------------------------------------------|
| C <sub>10</sub> H <sub>21</sub> NH <sub>2</sub>                | 77             | 113-130   | C <sub>23</sub> H <sub>44</sub> N <sub>2</sub> O <sub>4</sub> S |
| C <sub>12</sub> H <sub>25</sub> NH <sub>2</sub>                | 73             | 106-167   | C <sub>23</sub> H <sub>48</sub> N <sub>2</sub> O <sub>4</sub> S |
| C <sub>14</sub> H <sub>29</sub> NH <sub>2</sub>                | 66             | 111-181   | C <sub>27</sub> H <sub>52</sub> N <sub>2</sub> O <sub>4</sub> S |
| C <sub>14</sub> H <sub>29</sub> N <sup>+</sup> CH <sub>3</sub> | 72             | 100-124   | C <sub>25</sub> H <sub>54</sub> N <sub>2</sub> O <sub>4</sub> S |
| C <sub>6</sub> H <sub>13</sub> SH                              | 87             | 120-121   | C <sub>19</sub> H <sub>35</sub> NO <sub>4</sub> S <sub>2</sub>  |
| C <sub>8</sub> H <sub>17</sub> SH                              | 88             | 87-91     | C <sub>21</sub> H <sub>39</sub> NO <sub>4</sub> S <sub>2</sub>  |
| C <sub>10</sub> H <sub>21</sub> SH                             | 79             | 94-120    | C <sub>23</sub> H <sub>43</sub> NO <sub>4</sub> S <sub>2</sub>  |
| C <sub>12</sub> H <sub>25</sub> SH                             | 74             | 89-155    | C <sub>25</sub> H <sub>47</sub> NO <sub>4</sub> S <sub>2</sub>  |
| C <sub>16</sub> H <sub>33</sub> SH                             | 88             | 78-190    | C <sub>29</sub> H <sub>55</sub> NO <sub>4</sub> S <sub>2</sub>  |

The following example illustrates sensitizing of emulsions with sensitizers of the type listed above:

#### EXAMPLE 2

The compounds referred to in the preceding table were added in the amounts indicated in the following table to a high speed silver bromoiodide gelatino emulsion. The respective emulsions were coated onto a cellulose acetate support. A sample of each coating was exposed on an Eastman 1B sensitometer and were then processed for 5 minutes in Kodak Developer DK-50, fixed, washed and dried with the following results:

| Compound                                                       | g./Ag mole | Relative speed | γ    | Fog |
|----------------------------------------------------------------|------------|----------------|------|-----|
| Control                                                        | 100        | 1.02           | .15  |     |
| C <sub>14</sub> H <sub>29</sub> NH <sub>2</sub>                | .15        | 118            | 0.95 | .18 |
| C <sub>14</sub> H <sub>29</sub> NH <sub>2</sub>                | .75        | 209            | 0.84 | .29 |
| C <sub>14</sub> H <sub>29</sub> NH <sub>2</sub>                | 3.0        | 246            | 0.85 | .42 |
| C <sub>14</sub> H <sub>29</sub> N <sup>+</sup> CH <sub>3</sub> | .75        | 200            | 0.85 | .26 |
| C <sub>14</sub> H <sub>29</sub> N <sup>+</sup> CH <sub>3</sub> | 3.0        | 219            | 0.76 | .41 |
| Control                                                        | 100        | 0.99           | .12  |     |
| 15 bis*                                                        | .15        | 151            | 0.90 | .19 |
| bis*                                                           | .75        | 214            | 0.85 | .22 |
| bis*                                                           | 3.0        | 204            | 0.83 | .24 |
| Control                                                        | 100        | 1.02           | .14  |     |
| 20 C <sub>8</sub> H <sub>17</sub> SH                           | .75        | 151            | 0.90 | .16 |
| C <sub>8</sub> H <sub>17</sub> SH                              | 3.0        | 148            | 0.90 | .23 |
| C <sub>10</sub> H <sub>21</sub> SH                             | .15        | 135            | 0.90 | .16 |
| C <sub>10</sub> H <sub>21</sub> SH                             | .75        | 174            | 0.89 | .29 |
| C <sub>10</sub> H <sub>21</sub> SH                             | 3.0        | 166            | 0.83 | .57 |
| C <sub>10</sub> H <sub>21</sub> SH                             | .15        | 155            | 0.95 | .17 |
| C <sub>10</sub> H <sub>21</sub> SH                             | .75        | 162            | 0.87 | .39 |
| C <sub>10</sub> H <sub>21</sub> SH                             | 3.0        | 200            | 0.72 | .61 |
| C <sub>10</sub> H <sub>21</sub> NH <sub>2</sub>                | .15        | 115            | 0.98 | .12 |
| C <sub>10</sub> H <sub>21</sub> NH <sub>2</sub>                | .75        | 138            | 0.92 | .14 |
| C <sub>10</sub> H <sub>21</sub> NH <sub>2</sub>                | 3.0        | 166            | 0.96 | .23 |
| C <sub>12</sub> H <sub>25</sub> NH <sub>2</sub>                | .15        | 132            | 0.94 | .15 |
| C <sub>12</sub> H <sub>25</sub> NH <sub>2</sub>                | .75        | 224            | 0.87 | .25 |
| C <sub>12</sub> H <sub>25</sub> NH <sub>2</sub>                | 3.0        | 289            | 0.84 | .48 |
| C <sub>6</sub> H <sub>13</sub> SH                              | .15        | 107            | 1.05 | .12 |
| C <sub>6</sub> H <sub>13</sub> SH                              | .75        | 120            | 1.07 | .11 |
| C <sub>8</sub> H <sub>17</sub> SH                              | .15        | 120            | 0.99 | .12 |
| C <sub>8</sub> H <sub>17</sub> SH                              | .75        | 135            | 0.91 | .12 |
| C <sub>8</sub> H <sub>17</sub> SH                              | 3.0        | 159            | 0.94 | .16 |
| Control                                                        | 100        | 1.26           | .14  |     |
| C <sub>12</sub> H <sub>25</sub> SH                             | .15        | 151            | 1.11 | .15 |
| C <sub>12</sub> H <sub>25</sub> SH                             | .3         | 174            | 1.01 | .17 |
| C <sub>12</sub> H <sub>25</sub> SH                             | .75        | 200            | 0.98 | .33 |
| 50 bis A                                                       | .75        | 162            | 0.99 | .18 |
| bis A                                                          | 3.0        | 145            | 1.02 | .20 |
| bis B                                                          | .75        | 182            | 0.95 | .23 |
| bis B                                                          | 3.0        | 162            | 0.88 | .26 |

The designation under the heading "Compound" refers to the mercapto or amino compound which was reacted with the quaternary ammonium epoxide to form the sensitizer used. The designation "bis\*" refers to



which was used to prepare a bisquaternary ammonium sensitizer which was prepared as the perchlorate salt having the empirical formula C<sub>34</sub>H<sub>72</sub>Cl<sub>2</sub>N<sub>4</sub>O<sub>12</sub>S<sub>2</sub>. The designation "bis A" refers to (HSCH<sub>2</sub>CH<sub>2</sub>)<sub>2</sub>S, the bisquaternary ammonium sensitizer resulting therefrom having the empirical formula C<sub>30</sub>H<sub>52</sub>N<sub>2</sub>O<sub>8</sub>S<sub>2</sub>. The designation "bis B" refers to the dimercaptan HS(CH<sub>2</sub>)<sub>10</sub>SH from which the bisquaternary ammonium sensitizer having the empirical formula C<sub>36</sub>H<sub>64</sub>N<sub>2</sub>O<sub>8</sub>S<sub>4</sub>·2H<sub>2</sub>O was prepared. It was these resulting sensitizers which were used in obtaining the above data.

It is to be understood that the material designated "control" comprised an emulsion exactly comparable, similar-

ly processed, etc., to the emulsions of the invention except that the sensitizer referred to was not embodied therein.

The invention is useful for the sensitizing of various types of emulsions, which emulsions may or may not include various addenda. Some of the types of addenda which may be present in emulsions sensitized in accordance with our invention are the following:

(1) OPTICAL SENSITIZERS

If desired, the emulsions can be optically sensitized with cyanine or merocyanine dyes such as those described in any of the following patents: U.S. Patents Nos. 1,846,301, 1,846,302 and 1,942,854 of Brooker; U.S. Patent No. 1,990,507 of White; U.S. Patents Nos. 2,112,140, 2,165-338, 2,493,747 and 2,739,964 of Brooker and White; U.S. Patent No. 2,493,748 of Brooker and Keyes; U.S. Patents Nos. 2,503,776 and 2,519,001 of Sprague; U.S. Patent No. 2,666,761 of Heseltine and Brooker; U.S. Patent No. 2,734,900 of Heseltine; U.S. Patent No. 2,739,149 of Van Lare; and British Patent 450,958 of Kodak Limited.

(2) STABILIZERS

The mercury compounds of U.S. Patent No. 2,728,663 of Allen, Byers and Murray, U.S. Patent No. 2,728,664 of Carroll and Murray or U.S. Patent No. 2,728,665 of Leubner and Murray; gold salts as described in U.S. Patent No. 2,597,856 of Damschroder or U.S. Patent No. 2,597,915 of Yutzy and Leermakers; triazoles as described in U.S. Patent No. 2,444,608 of Heimbach and Kelly; azaindenes of U.S. Patents Nos. 2,444,605 and 2,444,606 of Heimbach and Kelly, U.S. Patents Nos. 2,450,397 and 2,444,607 of Heimbach, U.S. Patent No. 2,444,609 of Heimbach and Clark, U.S. Patents Nos. 2,713,541 and 2,743,181 of Allen and Reynolds, U.S. Patent No. 2,716-062 of Carroll and Beach, U.S. Patent No. 2,735,769 of Allen and Beiffuss, U.S. Patent No. 2,756,147 of Reynolds and Sagal, U.S. Patent No. 2,772,164 of Allen and Sagara or those referred to in the article by Birr in "Z. wiss Phot," volume 47, 1952, pp. 2-28; disulfides as disclosed in Belgian Patent No. 596,317; quaternary benzothiazolium compounds as listed in U.S. Patent No. 2,131,038 of Brooker and Staud; polymethylene bis-benzothiazolium salts as disclosed in U.S. Patent No. 2,694,716 of Allen and Wilson; zinc and cadmium salts as disclosed in U.S. Patent No. 2,839,405 of Jones; or a carbonylmethylmercapto compound as disclosed in U.S. Patent No. 2,819,965 of Murray, Reynolds and Van Allan.

(3) GELATIN PLASTICIZERS

Glycerin; dihydroxy alkanes such as 1,5-pentane diol as described in U.S. Patent No. 2,960,404 of Milton and Murray; esters of ethylene bis-glycolic acids such as ethylene bis-(methylglycolate) as described in U.S. Patent No. 2,904,434 of Milton; bis(ethoxy diethylene glycol) succinate as described in U.S. Patent No. 2,940,854 of Gray; or a polymeric hydrosol as results from the emulsion polymerization of a mixture of an amide of an acid of the acrylic acid series, an acrylic acid ester and a styrene-type compound as described in U.S. Patent No. 2,852,386 of Tong.

(4) HARDENERS

Formaldehyde; a halogen-substituted aliphatic acid such as mucobromic acid as described in U.S. Patent No. 1,080,019 of White; a compound having a plurality of acid anhydride groups or a dicarboxylic or a disulfonic acid chloride as described in U.S. Patents Nos. 2,725,294 and 2,725,295 of Allen and Carroll; a cyclic 1,2-diketone as described in U.S. Patent No. 2,725,305 of Allen and Byers; a bisester of methanesulfonic acid such as 1,2-di-(methane-sulfonyloxy)-ethane as described in U.S. Patent No. 2,726,162 of Allen and Laakso; 1,3-dihydroxy-methylbenzimidazol-2-one as described in U.S. Patent No. 2,723,316; a dialdehyde as described in application Serial No. 18,471, and now abandoned, of Allen and Burness; 75

a bis-aziridine compound as described in U.S. Patent No. 2,950,197 of Allen and Webster; a 2,3-dihydroxy dioxane as described in U.S. Patent No. 2,870,013 of Jeffreys; or a diisocyanate as described in application Serial No. 805-357 and now Patent No. 3,103,437 of Henn et al.

(5) COATING AIDS

Saponin; an acylated alkyl taurine as described in U.S. Patent No. 2,739,891; a water-soluble maleopimarate as described in U.S. Patent No. 2,823,123; or an alkali metal salt of a substituted amino acid as described in Knox and Wilson application Serial No. 600,679 and now Patent No. 3,038,804.

The addenda which we have described may be used in various kinds of photographic emulsions such as X-ray or other non-optically sensitized emulsions or in orthochromatic, panchromatic or infrared sensitive emulsions. They may be added to the emulsion before or after sensitizing dyes have been provided. Various silver salts may be used as the light-sensitive salts in the emulsion, such as silver bromide, silver iodide, silver chloride or mixed silver halides such as silver bromochloride or silver bromoiodide. The agents may be used in emulsions intended for color photography, for example emulsions containing color-forming couplers or emulsions to be developed by solutions containing couplers or other color-generating materials. Emulsions of the mixed packet type as described in U.S. Patent No. 2,698,794 or emulsions of the mixed grain type as described in U.S. Patent No. 2,592,243 may be sensitized in accordance with the invention. The sensitizers of the invention may be used in emulsions for color purposes having incorporated couplers with reversal as well as direct color development.

I claim:

35 1. A silver halide photographic emulsion containing therein, per mole of silver halide, 0.1 to 4 g. of a sensitizer selected from the group consisting of the compounds having the formula



wherein Y is selected from the group consisting of alkyl mercapto groups of 6-30 carbon atoms and secondary and tertiary amino groups containing linear chains of 45 10-30 carbon atoms, R is lower alkyl of 1-4 carbon atoms and X is a suitable anion and the compounds having the formula



50 wherein R is lower alkyl of 1-4 carbon atoms, X is a suitable anion and Z is selected from the group consisting of dimercapto and diamino groups in which the mercapto and the amino groups are joined by an alkylene chain containing at least 4 carbon atoms and dimercapto 55 and diamino groups in which the mercapto and the amino groups are joined by an aliphatic chain of hetero atoms including at least 4 carbon atoms.

55 2. A silver halide photographic emulsion containing, per mole of silver halide, 0.1 to 4 g. of a sensitizer having the formula



60 wherein Y is a secondary amine group, having the formula  $C_{10}H_{21}NH-$ , R is lower alkyl of 1-4 carbon atoms and X is a suitable anion.

65 3. A silver halide photographic emulsion containing, per mole of silver halide, 0.1 to 4 g. of a sensitizer having the formula



70 wherein Y is a secondary amine group having the formula  $C_{12}H_{25}NH-$ , R is alkyl of 1-4 carbon atoms and X is a suitable anion.

4. A silver halide photographic emulsion containing,

per mole of silver halide, 0.1 to 4 g. of a sensitizer having the formula



wherein Y is an alkyl mercapto group having the formula  $C_8H_{17}S-$ , R is alkyl of 1-4 carbon atoms and X is a suitable anion.

5. A silver halide photographic emulsion containing, per mole of silver halide, 0.1 to 4 g. of a sensitizer having the formula



wherein Y is an alkyl mercapto group having the formula  $C_{16}H_{33}S-$ , R is alkyl of 1-4 carbon atoms and X is a 15 suitable anion.

6. A silver halide photographic emulsion containing as a sensitizer therein, per mole of silver halide, 0.1 to 4 g. of 3-n-dodecylamino-2-hydroxypropyltrimethylammonium p-toluene-sulfonate.

7. A silver halide photographic emulsion containing as a sensitizer therein, per mole of silver halide, 0.1 to 4 g. of a sensitizer having the formula



in which Z is



R is alkyl of 1-4 carbon atoms and X is a suitable anion.

5. A silver halide photographic emulsion containing therein, per mole of silver halide, 0.1 to 4 g. of a sensitizer having the formula



10 in which Z is  $-S(CH_2)_{10}S-$ , R is alkyl of 1-4 carbon atoms, and X is a suitable anion.

9. A silver halide photographic emulsion containing therein, per mole of silver halide, 0.1 to 4 g. of a sensitizer having the formula



in which Z is  $-SCH_2CH_2SCH_2CH_2S-$ , R is alkyl of 1-4 carbon atoms and X is a suitable anion.

20

References Cited by the Examiner

UNITED STATES PATENTS

2,940,851 6/40 Beavers et al. ----- 96-107  
3,038,805 6/62 Dann et al. ----- 96-107

25

NORMAN G. TORCHIN, Primary Examiner.